

July 10, 1923.

1,461,178

H. S. COOPER

ALLOY

Filed Aug. 26, 1918

FIG. 1



FIG. 2



FIG. 5



FIG. 3



FIG. 4



FIG. 6



Witness  
Geo. F. Fischer,

Inventor

Hugh S. Cooper

By

*Fischer & Moore*

Attorneys

Patented July 10, 1923.

1,461,178

# UNITED STATES PATENT OFFICE.

HUGH S. COOPER, OF CLEVELAND, OHIO, ASSIGNOR, BY MESNE ASSIGNMENTS, TO  
KEMET LABORATORIES COMPANY INC., A CORPORATION OF NEW YORK.

## ALLOY.

Application filed August 26, 1918. Serial No. 251,375.

*To all whom it may concern:*

Be it known that HUGH S. COOPER, a citizen of the United States, residing at Cleveland, in the county of Cuyahoga and State of Ohio, has invented certain new and useful Improvements in an Alloy, of which the following is a specification.

This invention pertains to an alloy comprising the elements silicon, aluminum and nickel, the silicon and aluminum being present in relatively small amounts and the nickel in a preponderating amount. To these elements there may be added either tungsten or molybdenum or both tungsten and molybdenum, but primarily my object is to mix nickel, silicon and aluminum in the most suitable proportions to produce an alloy of relatively low cost which shall be neither too soft nor too brittle for special services but shall possess, on account of the properties of the component metals and the chemical combinations formed, several valuable characteristics, namely: toughness, non-corrodibility, a low melting point and extreme hardness at a red heat. The properties of red-hardness, toughness, and a low melting point are very desirable for the manufacture of castings of all kinds, particularly cutting tools, while the non-corrodible feature is highly desirable where the alloy is used for valves, valve-seats, crucibles, annealing boxes, etc. Thus the alloy is of great utility in the manufacture of dies of all kinds, draw rings for shell forgings and wire dies, engine valves, ornamental objects, weights, etc., and to illustrate the value of the property of red-hardness, dies and draw rings made of this alloy when subjected to hot work will last in most cases approximately ten times as long as other materials now in use. Furthermore, the alloy requires no heat treatment, inasmuch as a permanent hardness is produced by the silicides which are present in the alloy.

Where the alloy is used for ornamental objects it may be highly polished and the luster will be retained for some time. A beautiful blending of colors may also be produced on the surface of the alloy by subjecting the same at a red heat to a blast of air. These colors are produced by the various elements in the alloy and are characteristic of silicides.

In the accompanying sheet of drawings, Figs. 1 to 6 show six charts or graphic rep-

resentations of the hardness curves of various silicon-nickel, aluminum-nickel, and aluminum-silicon-nickel alloys, and Figs. 2 and 4 are substantially identical to the two charts shown in my application for Letters 60 Patent filed Feb. 23, 1918, Serial Number 218,791, now U. S. Patent No. 1,278,304 wherein I disclose the hardness curves of certain alloys of aluminum and nickel; and aluminum, silicon and nickel. However, it 65 should be noted that the charts in the application referred to show alloys in which the proportions require the use of zirconium to produce a satisfactory high-speed cutting-tool alloy, whereas Figs. 3 and 6 in the present application show alloys without zirconium or chromium, which as ternary alloys possess the characteristics and valuable properties herein stated.

Now referring more particularly to Fig. 75 1, this chart is submitted to show a binary series of silicon-nickel, wherein less than ten (10) percent of silicon has proven to be too soft for the service in view, although possessed of a fair degree of toughness. This 80 chart also shows that an alloy of silicon and nickel containing more than ten (10) percent of silicon within the limits given, while sufficiently hard, is quite too brittle for satisfactory service. The same objections were 85 found in the binary series of aluminum-nickel, shown in Fig. 2, except that the alloys containing more than ten (10) percent of aluminum are not quite as hard as alloys with a corresponding amount of silicon, and 90 with more than ten (10) percent of aluminum the alloys are extremely crystalline and very fragile.

However, a remarkable change takes place 95 when aluminum, silicon and nickel are mixed in certain definite proportions; that is, I have found by careful experimentation (as indicated in the charts Figs. 3 to 6, inclusive,) that it is possible to produce alloys of these three metals without the addition of 100 another metal which are extremely hard at the same time very tough and possessive of a high tensile strength, and having a fine grain similar to rolled steel. I have also found that to give this combined hardness, 105 toughness and strength there must be present in the alloy a preponderating amount of nickel or cobalt and not less than three (3) percent each of aluminum and silicon, nor more than twelve (12) percent aluminum 110

and eight (8) percent silicon. Furthermore, in order to produce the desired results and gain the main object in view, I prefer the alloys containing an excess of aluminum over silicon, as these are the toughest and strongest with equal hardness. Those containing more than eight (8) percent silicon are rather brittle, therefore less desirable.

Alloys of preferred composition for cutting tools, draw rings, dies, etc., contain approximately seven (7) percent silicon; seven (7) percent aluminum, eighty-six (86) percent nickel, see the dotted sector bearing the terms "hard and tough" in Fig. 6. A slightly harder alloy, but one not quite as tough, contains about eight (8) percent aluminum; six (6) percent silicon; eighty-six (86) percent nickel. The best composition that I have so far discovered for cutting tools contains ten (10) percent aluminum; five (5) percent silicon, and eighty-five (85) percent nickel, see Fig. 3. This particular alloy easily cuts glass and will withstand severe blows with a hammer without fracture. If one (1) percent aluminum is added to this best composition (see Fig. 3), with the silicon remaining at approximately five (5) percent, the hardness is slightly increased and the toughness decreased, making the alloy suitable for cutting cast iron, but without sufficient toughness to be used on steel. This last named alloy represents approximately the limit in percentage of aluminum, with five (5) percent silicon, for with higher percentages of aluminum, it becomes extremely brittle compared with the alloys of the more desirable proportions in Figs. 3 and 6. Nevertheless, the proportions of elements within the limits given in Figs. 3 to 40 6, which do not yield the combined hardness and toughness desired for cutting tools, etc., have value and utility in making cast crucibles and other articles which must be non-corrodible and have the property of resisting 45 powerful acids. Briefly, the silicon and aluminum impart to the nickel an increased resistance to acid and other corrosive influences. These alloys moreover, have been found to be non-scaling and resistant to 50 oxidizing influences at high temperatures (800-1100° C.), a protective coating apparently being formed by slight oxidation, which does not however penetrate the body of the metal.

55 The ternary alloys described herein are considerably toughened, and the red-hardness greatly increased by the addition of tungsten from one-half ( $\frac{1}{2}$ ) to about twenty-five (25) percent; and small amounts of molybdenum may also be added to increase the hardness and toughness. If tungsten is present in quantities over ten (10) percent, the molybdenum need not exceed about five (5) percent, and if the tungsten is less than ten (10) percent the molybdenum may be

present up to an equal amount with tungsten. If no tungsten is used, molybdenum may be used up to about twenty-five (25) percent, and for the purposes of the present invention, these two metals may be considered equivalents and the appended claims are to be so construed. Tungsten and molybdenum, if used, displace the nickel.

The red-hardness which is a property of these alloys is probably due to the complex 75 silicides which are formed in the ternary alloys, these being still further improved on adding tungsten or molybdenum by the formation of the silicides of tungsten and molybdenum, which are known to be very 80 stable at high temperatures.

To obtain these alloys I weigh out the specified amounts of metallic silicon, aluminum and nickel, preferably in the form of shot, and place the aluminum and silicon in the bottom of a crucible and cover them with the nickel. The temperature of the furnace need not be brought to the melting point of nickel as the combination of aluminum and nickel takes place at a point about 90 midway between the melting points of aluminum and that of nickel. A great amount of heat is given off by combination of these two metals, which is sufficient to raise the temperature to a white heat. 95 When this reaction ceases the tungsten or molybdenum may be added in the form of powder or high grade ferro. The alloy is then stirred and the heating continued until the added metals have been dissolved. 100

If ferro-tungsten or ferro-molybdenum are used the alloy will contain appreciable amounts of iron. These small amounts of iron seem to have no detrimental effect. The ferro alloys are more easily obtained 105 and are somewhat cheaper than the powdered metal; therefore, it is sometimes of advantage to use ferro alloys in place of the respective powdered metals.

What I claim is:

1. An alloy composed of a preponderating amount of nickel, aluminum and silicon in which the percentage of either of the last two substances is not less than three percent and not more than twelve percent. 110
2. An alloy, comprising a preponderating amount of nickel and not less than three percent each of aluminum and silicon nor more than twelve percent aluminum and eight percent silicon. 115
3. An alloy having a scleroscopic hardness above sixty, containing mainly nickel, together with three to twelve percent aluminum and three to eight percent silicon. 120
4. An alloy, containing approximately eighty-two to eighty-six percent nickel, six to twelve percent aluminum, and five to eight percent silicon, the three elements combined having a scleroscopic hardness approximating sixty or higher. 125

5. An alloy composed of a preponderating amount of nickel, aluminum not less than three percent nor more than twelve percent, silicon not less than three percent nor more than eight percent, and the amount of aluminum being not less than the amount of silicon.
6. An alloy composed of a preponderating amount of nickel, aluminum not less than three percent nor more than twelve percent, silicon not less than three percent nor more than eight percent, and the aluminum being in excess of the silicon.
7. An alloy, comprising approximately ten percent aluminum, five percent silicon, and a preponderating amount of nickel up to eighty-five percent.
8. An alloy composed of a preponderating amount of nickel, one half to about twenty-five percent of tungsten, three to twelve percent of aluminum and five to eight percent of silicon.
9. An alloy composed of a preponderating amount of nickel, tungsten and molybdenum not exceeding together twenty-five percent and the amount of molybdenum not exceeding the amount of tungsten, aluminum three to twelve percent and silicon three to eight percent.

Signed at Cleveland, in the county of 30  
Cuyahoga, and State of Ohio, this 22nd day  
of August, 1918.

HUGH S. COOPER.